

April 28, 1970

G. L. HERWIG ET AL

3,508,908

PRODUCTION OF ALUMINUM AND ALUMINUM ALLOYS

Filed Sept. 6, 1966



**1**

3,508,908

**PRODUCTION OF ALUMINUM AND ALUMINUM ALLOYS**

George Lang Herwig, East Brighton, Victoria, and Ernest Foley, East Burwood, Victoria, Australia, assignors to Conzinc Riotinto of Australia Limited, Melbourne, a corporation of Victoria, and Commonwealth Scientific and Industrial Research Organization, Victoria, Australia, a body corporate of Australia

Filed Sept. 6, 1966, Ser. No. 577,473

Claims priority, application Australia, Sept. 8, 1965, 63,759/65; Aug. 29, 1966, 10,290/66  
Int. Cl. C22b 21/02; C22d 3/12

U.S. Cl. 75—68

20 Claims

**ABSTRACT OF THE DISCLOSURE**

A process for the production of aluminum and aluminum alloys wherein a fused salt electrolyte containing at least one alkali metal halide is electrolyzed using a cathode of a molten metal or alloy, in which the electrolyte comprises a halide of a metallic reductant for aluminum chloride which reductant is soluble in the cathode, the metallic reductant being deposited by electrolysis from the electrolyte and dissolved in the cathode, and the cathode metal or alloy and the contained reductant being brought into contact with a double salt of alchlor.

This invention relates to the production of aluminum and aluminum alloys from aluminum chloride (hereinafter referred to as alchlor) or from salts containing alchlor, and refers especially to a process of and apparatus for reducing a salt containing alchlor to aluminum by reaction with a metal reductant which may, for example, be magnesium. The invention also includes a process and apparatus for the production of aluminum by fusion electrolysis using alchlor as the feed material.

The alchlor is preferably used in the form of a double salt, for example a low melting point double salt containing sodium chloride and alchlor.

It will be appreciated that, depending on whether the amount of alchlor present in the salt phase is equal to or is greater or less than the stoichiometric proportion, there will be present either a true double salt or a solution of alchlor in a salt. The term "double salt" is used in the specification and claims hereof to include either (a) a double salt of alchlor and the halide of an alkali metal or (b) a solution of alchlor in a salt or salt phase.

The invention broadly resides in a process for the production of aluminum and aluminum alloys which comprises reacting a metallic reductant with a double salt of alchlor.

In one form of the invention molten magnesium is reacted with a molten double salt of sodium chloride and aluminum chloride. Some advantages of using the double salt are the ease of handling and the relatively low vapour pressure of aluminum chloride above the salt at temperatures in the vicinity of 750° C. (i.e. above the melting point of aluminum).

It is advantageous to add a proportion of the circulating aluminum or aluminum-magnesium alloy to the molten magnesium to ensure that the density of the metallic phase at all times is greater than that of the molten saline phase.

The reaction may be carried out in a reactor associated with an electrolytic cell in which case the magnesium chloride formed by the reaction may be treated electrolytically for recovery of magnesium and chlorine.

Electrolytic processes for the production of aluminum which are in present day use employ aluminum oxide as a solution in a double salt of sodium and aluminum

**2**

fluorides. Disadvantages of this system include (1) the consumption of high purity carbon electrodes by the oxygen component of the feed material at a rate which varies from 0.6 to 1.0 lb. of carbon per lb. of aluminum produced; (2) the low voltage efficiency of the cell of 35 to 45% which results from a summation of high voltage drops across the anode which must be adapted to continuous feeding, across the carbon lining which must be thick to contain the high temperatures within the cell, across the polar gap which must be large to allow clearance between the distorted cathode metal surface and the anode, and finally due to polarisation effects on the anode as a result of intermittent charging and variation of electrolyte compositions; (3) losses of expensive electrolyte by vapourisation occasioned by the open top construction of the cell necessitated by the need to intermittently and evenly feed solid alumina to the electrolyte; (4) severe corrosion and low cell life resulting from the high cell temperature of 950 to 1000° C., and (5) an appreciable labour requirement for introducing feed material.

The art contains records of attempts to produce aluminum from anhydrous alchlor by electrolysis of an electrolyte composed of alchlor dissolved in certain fused metal halides. A number of disadvantages have prevented commercial acceptance of such processes. Alchlor is a volatile solid subliming at about 178° C. Although its vapour pressure may be lowered substantially in molten alkali metal chloride baths, alchlor is readily distilled from such baths when operating at or about the melting point of aluminum (661° C.). As a consequence these processes are operated at low temperatures or under a positive pressure. Eutectic or low melting point fused salt mixtures containing alchlor have very poor electrical conductivity, especially below the melting point of aluminum. At the operating temperatures of such processes molten solutions of alchlor are corrosive towards graphite and carbon which are essentially the only practical anode materials which can withstand and co-produced chlorine. At low temperatures aluminum is deposited as a solid commingled with electrolyte which is inconvenient to separate from the metal crystals, and cell voltages at practical current densities are very high. At high temperatures cell voltages can be reduced and liquid metal obtained but the pressurised equipment is expensive and corrosion is severe.

Our invention in one of its aspects seeks to overcome the disadvantages of processes using electrolytes containing alchlor, while retaining the advantages of alchlor as a feed material, by providing a process wherein little, if any, alchlor can ever be present in the electrolyte.

According to this aspect of the invention a process for the electrolytic production of aluminum and aluminum alloys comprises electrolyzing a fused salt electrolyte containing at least one alkali metal halide using as cathode a molten metal or alloy, which molten metal or alloy contains in solution a metallic reductant deposited from the electrolyte, and contacting the molten metal or alloy and the contained metallic reductant with a double salt of alchlor or with a solution of alchlor in a molten salt.

In addition to alkali metal halides the electrolyte may contain one or more alkaline earth metal halides and/or rare earth metal halides.

Preferably the alchlor is contacted with the molten metal or alloy in such a manner that there is negligible alchlor entering the electrolysis compartment.

More particularly the invention includes a process for the electrolytic production of aluminum which comprises electrolyzing in an electrolysis compartment or cell a fused salt electrolyte containing an alkali metal halide, the cathode being molten aluminum or aluminum alloy containing a metallic reductant deposited from the elec-

trolyte by the electrolysis, transferring the molten aluminum or aluminum alloy and reductant to a reactor compartment or vessel, reacting alchlor with the metallic reductant in the reactor compartment or vessel, transferring the chloride product of the metallic reductant to the electrolysis compartment or cell, re-cycling molten aluminum containing a lower concentration of the metallic reductant back to the electrolysis compartment or cell, and discharging the molten metal product from the reactor compartment or vessel.

Again the electrolyte may contain one or more alkaline earth metal halides and/or rare earth metal halides in addition to the alkali metal halide.

According to another aspect of the invention, an important feature resides in effecting the reaction between the metallic reductant and the alchlor which latter is preferably in the vapour state, in a compartment or vessel which is distinct or separate from the electrolysis compartment, so that little or no alchlor is permitted to enter the electrolysis compartment and consequently the possibility of its loss with and contamination of the chlorine produced in the electrolysis, and the attack by the alchlor on the anode material, are substantially prevented.

Preferably the reaction between the metallic reductant and the alchlor is effected in a two-stage reactor compartment or vessel, wherein a salt phase capable of absorbing alchlor as a double salt simultaneously contacts both the alchlor as vapour and the molten aluminum containing a metallic reductant. In this case a reaction occurs between the reductant and the alchlor double salt which results in a lowering of reductant concentration in the aluminum. The aluminum from the first stage is re-cycled to the electrolysis compartment and the salt phase containing both the chloride product of the reductant and alchlor to saturation as a double salt or solution is contacted in a second stage to react to or approaching extinction with fresh molten aluminum and reductant from the electrolysis compartment.

The aluminum from the second stage passes back to the first stage while the salt phase containing the chloride product of the reductant but now denuded of alchlor is re-cycled to the electrolysis compartment.

In one form of the invention a small portion of the electrolyte may be used as the alchlor-absorbing salt phase, the portion of electrolyte being metered at such a rate to the first stage as to ensure that the salt phase leaving the second stage contains negligible amounts of alchlor.

Depending upon the degree to which it is desired to reduce the reductant content of the metal being re-cycled to the electrolysis compartment or cell two or more stages of contact may be used, in all cases alchlor being fed only to the first stage. The two or more stage counter-current reaction between the reductant electro deposited into the re-cycled aluminum and the alchlor double salt ensures that the salt phase leaving the reactor which is re-cycled to the electrolysis compartment is essentially free of alchlor by last being in contact with an excess of reductant. The aluminum working back to the first stage then still has a content of reductant sufficient for further reaction in this stage.

In the first stage the salt phase is continuously in contact with the alchlor vapour and absorbs it as fast as the alchlor portion of the double salt reacts with the excess reductant. Thus the salt phase leaves the first stage for the later stages still with a content of alchlor to be removed by incoming reductant. The quantity of alchlor reacted overall will be equivalent to the quantity of reductant removed in the reactor, firstly, because there will be a quantity of reductant in the first stage to react with the alchlor vapour being fed in, and secondly because the reductant present in the second stage will react with the alchlor (present as a double salt) to or approaching extinction. This is ensured by metering the fresh electrolyte into the first stage at a suitable rate when the reductant

is an alkaline earth metal. If an alkali metal is used as reductant it is not necessary to pass a portion of the electrolyte through the reactor system as the chloride product forms the necessary double salt with alchlor and the quantity flows are self-adjusting.

When the above quantity requirements are met some excess reductant will exist in the first stage to react with the alchlor in the double salt present. Further alchlor vapour can then absorb into the double salt.

Overall the quantity of alchlor vapour absorbed into the double salt must essentially equal the quantity of reductant reacted out of aluminum which is the quantity of reductant produced in the electrolysis compartment. Therefore, for the successful operation of the process of the invention it is not necessary for the electrolysing current and rate of input of alchlor vapour to be in continuous and exact synchronisation. The system can only absorb alchlor vapour as fast as it can react, that is as fast as reductant is produced and fed to the reactor, and it can be adapted readily to automatic control of alchlor vapour input.

In the case of an alkali metal reductant, alchlor cannot enter the electrolysis compartment in any appreciable quantity. Alchlor can only leave the first stage of the

reactor as a double salt and this can only be produced if reductant is reacted to the chloride in this stage. It follows that an excess of reductant must always exist in the later stages which will be capable of reacting essentially all of the alchlor out of the double salt. In the case of an alkaline earth metal reductant electrolyte is metered into the first stage to form a double salt with the alchlor, the quantity metered being such as to achieve the above requirements.

In both cases not only are losses of alchlor via the electrolysis compartment substantially avoided, but additionally contamination of the halogen co-product and attack by the alchlor on the anode are either prevented or are of negligible degree.

The metallic cathode should comprise a metal or alloy which is molten within the required temperature range, which is a sufficiently good solvent for the metallic reductant used and which is substantially unreactive to alchlor. Aluminum or an alloy of aluminum is preferably used. A preferred feature of the invention is the employment, as components of the fused salt electrolyte, of an alkali metal halide or mixture of alkali metal and alkaline earth metal halides.

The composition of the fused electrolyte should desirably be such that the metal or metals deposited at the cathode during electrolysis (i.e. the metallic reductant) have adequate solubility in the molten metallic cathode (e.g. in molten aluminum or aluminum alloy), low solubility in the saline phase, and, when dissolved in the molten cathode metal, have sufficient reactivity to reduce alchlor vapour.

As previously stated, the metallic reductant is transferred to a reactor compartment, distinct from the electrolysis compartment, wherein chemical interaction occurs between the metallic reductant and alchlor double salt. By this arrangement it becomes possible to control the amount of reductant to any level deemed necessary to ensure the desired degree of interaction. Contrary to what might be expected we have found that alchlor double salts will reduce the magnesium content of an aluminum magnesium alloy to extremely low values (e.g. 0.005%) at high efficiency, and hence magnesium by best fulfilling the above requirements is the preferred metallic reductant.

A further requirement of the fused electrolyte is that it must contain a salt capable of forming a double salt complex with alchlor under the temperature conditions of the reactor. Alkali metal halides fulfill this requirement in a satisfactory manner and preferably sodium or potassium chloride should constitute at least one component of the electrolyte.

However, the invention also includes the use of other

alkaline earth metals (e.g. calcium) and lithium as the metallic reductant, and the use of other alkaline earth metal halides or alkali metal halides, and in particular mixtures thereof, as components of the fused salt electrolyte.

Magnesium chloride, or other alkali earth metals, are used in admixture with the halides of sodium, potassium or other alkali metals. As a source of both reductant and complexing agent, alkali chlorides may be used alone or in admixture with each other.

Other alkali metal or alkaline earth metal halides, specifically the chlorides and/or fluorides, may be added, within the limitations set out above, to modify and improve the properties of the electrolyte.

In the preferred process of the invention a molten salt comprising either;

- (a) magnesium chloride admixed with halides of sodium and/or potassium, or
- (b) lithium chloride alone or admixed with halides of sodium and/or potassium,

is electrolysed in an electrolysis compartment using a dependent graphite or carbon anode and a molten aluminum cathode, the relative densities of the liquid phases being such that the molten cathode remains as a discrete phase at the bottom of the electrolytic cell. Under such conditions substantially pure chlorine is evolved from the anode and corresponding amounts of reductant dissolve in the aluminum cathode.

The aluminum plus reductant metal formed is transferred to a separate second compartment where it is reacted countercurrently with alchlor double salt under conditions of high, but not necessarily 100% efficiency. Aluminum or aluminum alloy denuded in reductant is collected in suitable collection equipment from which it is either recycled to the electrolysis compartment to maintain the cathode metal at the desired level or tapped off, as required.

The temperature at which the electrolysis and reduction processes are carried out is desirably maintained at 10-100° C. above the melting point of the electrolyte, or the cathode metal or the salt phase following the reduction process whichever is the highest.

A further feature of one form of the invention resides in enclosing the reactor compartment in such a manner that back pressure in the vapour or gas space is used to control the rate of alchlor addition; preferably the reactor compartment is totally enclosed to the gas phase, so that if an excess of alchlor is fed it accumulates as a gas and builds up pressure within the compartment. If the alchlor supply to this compartment is only at low pressure, then the accumulated pressure in the compartment retards or stops the flow of alchlor into the compartment and this state continues until sufficient of the excess alchlor vapour is consumed by fresh reductant contained in the liquid metal received from the electrolytic cell to reduce the back pressure and allow further flow. This is a very desirable feature as the alchlor feed rate is thereby automatically controlled according to demand.

Whereas the normal method of alloy manufacture would be to add the alloying element directly to the metal stream in most instance, where an alloying element forms a volatile chloride, the alloy may be produced by introducing the chloride of the element in addition to alchlor into the reactor compartment at the appropriate rate.

The process of this invention has a number of advantages over existing processes for the electrolytic production of aluminum. It consumes virtually no carbon, continuously produces aluminum at high current efficiencies and enables operation at temperatures above the melting point of aluminum yet significantly below those used in current aluminum extractive technology. By the use of gaseous alchlor a high purity feed can be introduced and

a closed cell construction used with several attendant advantages.

Important advantages derive from the introduction of the gaseous alchlor in a separate compartment to the electrolysis, in that a wide selection of cell electrolytes is possible and a composition can be used which gives high conductivity and low specific gravity. Resulting from this, high current densities are possible, close electrode spacing can be used and voltage drop across the electrolyte can be minimised. Fixed anodes of optimum design can be used with a low voltage drop across them. Similarly cathode connector design can be improved to reduce voltage drop at this point. Cell designs are possible which are amenable to automation so that routine labour and supervision requirements are reduced to a minimum.

Because aluminum compounds are not directly electrolysed, but instead a metal reductant is deposited as a solution in a flowing stream of aluminum or aluminum alloy, problems such as cathode over-potential and fog formation are substantially reduced and high voltage and current efficiencies are possible. By recycling the aluminum at a sufficient rate to ensure that the solution of reductant in the molten cathode is relatively diluent, the higher voltages required for decomposition of the reductant salt in the electrolyte rather than of alchlor are largely offset by the reduced activity of the reductant dissolved in the molten cathode.

We have determined that substantially all the aluminum present originally in the molten salt mixture may be removed by the use of only a small excess of metallic reductant. We have also determined that the use of a small excess of aluminum chloride in a molten salt will remove the reductant metal from the metallic product.

Examples of the operation of the process of this invention are as follows:

#### EXAMPLE 1

A fused salt electrolyte comprising 20% w./w. magnesium chloride 40% w./w. lithium chloride and 40% w./w. sodium chloride was electrolysed at 670°-700° C. in an alumina-lined cell fitted with a vertical carbon rod as anode and having a pool of commercial-grade aluminum as cathode. The interpolar gap was 0.71 inch, the current density 1080 amps per square foot and the overall voltage 3.2 to 3.4 volts.

After electrolysing for one hour the magnesium chloride content was replenished to 25% by adding additional molten magnesium chloride. Electrolysis was then continued for a further period of one hour after which the aluminum metal product was removed and on analysis was found to contain 3.97% w./w. metallic magnesium.

#### EXAMPLE 2

A reaction crucible was prepared by lining a mild steel crucible with high alumina refractory material. The crucible was fitted with a vertical shaft carrying an impeller at its lower end. 1,700 gms. of an aluminum-magnesium alloy, containing 6.5% magnesium, were added to the crucible followed by 500 gms. of sodium chloride, the quantity of alloy being selected to cause the interface between the metal and the salt phase, in the molten state, to pass through the impeller.

The crucible and contents were placed in a steel retort, evacuated, filled with argon and then heated to 750° C. Pure gaseous aluminum chloride was then fed in at a controlled steady rate (1.5 litres per minute S.T.P.) to the atmosphere above the salt phase. At the same time the impeller was rotated to splash molten metal onto the wall of the crucible and thereby increase the contact between the molten metal and the salt at the interface. The aluminum chloride was rapidly absorbed by the sodium chloride to form a double salt (sodium aluminum chloride) and the contact between the double salt and the aluminum-magnesium alloy at the interface resulted in a reaction between the double salt and the magnesium to yield magnesium chloride and to return sodium chloride

to the salt phase for absorption of further quantities of aluminum chloride.

When a very slight excess over the stoichiometric amount of aluminum chloride had been added to the apparatus, feeding of the aluminum chloride was discontinued and the apparatus was allowed to cool. The resulting ingot of aluminum was dense, free from chloride inclusions, and contained approximately 0.002% of magnesium.

In one method of operating the process continuously the metal reductant, magnesium, is fed at a known rate into the upper section of a vertical reactor containing molten aluminum and fused sodium chloride. Gaseous aluminum chloride is fed under pressure into the upper part of the reactor at a rate stoichiometrically equivalent to that of the magnesium. Product metal is drawn off from the base of the reactor at a corresponding rate, whilst magnesium chloride overflows a weir at the top of the reactor and may be diverted to an electrolytic cell for regeneration of magnesium and chlorine.

To facilitate the chemical reactions the contents of the reactor are continuously agitated.

To minimise the effect of fluctuations in the rate of flow of reactants it is found convenient to maintain a reserve of magnesium in the main metallic phase, this section being recirculated from a point a short distance above the product tapping point. Makeup magnesium may be added to the system as an alloy or pure metal may be blended into the recirculating stream.

We have found that aluminum chloride even in molten admixture with various other chlorides will react with sufficiently electro-positive metals at high efficiency, producing molten aluminum containing if so desired, only trace amounts of the metallic reductant.

We have demonstrated, however, that the position of equilibrium in this reaction is such that substantially all the aluminum chloride present originally in the molten salt mixture may be removed by the use of only a small excess of metallic reductant. We have also shown that the use of a small excess of aluminum chloride in a molten salt will remove the reductant metal from the metallic product.

#### EXAMPLE 3

85 gms. of magnesium ingot in a fused alumina crucible (8" x 3" diameter) were heated to 700° C. under an argon atmosphere in a steel crucible. Lumps of a double salt of aluminum and sodium chlorides (74.8% aluminum chloride) were added as required to maintain the temperature in the range of 750° to 800° C. until a total of 592 gms. had been added, agitating continuously with a tantalum stirrer. After cooling, the solid saline and metallic phases were separated mechanically and analysed. The magnesium content of the metallic aluminum phase was less than 0.004%. The aluminum chloride content of the saline phase ranged from 16.6% to 20%.

#### EXAMPLE 4

527.5 gms. of an aluminum-magnesium alloy (90.4% magnesium) were heated to 700° C. as described in the Example 3, after which 289 gms. of a double salt of sodium and aluminum chlorides (73.7% aluminum chloride) were added progressively with stirring. After cooling and separating the two phases, 517.5 gms. of aluminum were obtained with a magnesium content of 0.004 to 0.04%; the 274 gms. of saline phase contained 3.1 to 3.7% aluminum chloride.

The preceding Examples 3 and 4 demonstrate the effectiveness of this invention in the batchwise production of aluminum. There are advantages attached to carrying out the process in a continuous manner. This can readily be achieved, using general procedure of countercurrent flow in suitably designed contactors.

The form of apparatus for carrying out the invention, which is shown diagrammatically in the accompanying drawings, will now be described. These drawings

and the description thereof are illustrative only, and are in no way to be regarded as limitative of the invention. In the drawings the same reference numerals are used to refer to like or corresponding parts.

In the drawings: FIGURE 1 is a view in sectional elevation of apparatus for the electrolytic production of aluminum;

FIGURE 2 is a sectional view taken on line 2—2 of FIGURE 1; and

FIGURE 3 is a sectional plan view taken on line 3—3 of FIGURE 1.

The apparatus indicated generally at 1 is provided with an outer shell 2 which is thermally insulated by the lining 3. An inner graphite and/or carbon lining 4 contains the contents of the apparatus and carries current from the connectors 6 to the cathodic liquid metal layer 7. The sides of the electrolysis compartment or cell 11 are electrically insulated by a refractory lining 5.

The apparatus 1 is divided internally by graphite and/or carbon wall 8 and by graphite carbon and/or refractory wall 9 into five compartments, namely the electrolysis compartment 11, the pump compartment 12, the first stage reactor compartment or vessel 13, the second stage reactor compartment or vessel 14 and the product metal storage sump 15. The electrolysis compartment 11 contains a molten salt electrolyte 16 which is of lower specific gravity than the cathodic metal layer 7 therebeneath. Anodes 17, 18 preferably of graphite or carbon depend into the electrolyte 16 and are secured to the cover 19, the anode connection being indicated at 20. The undersurface of the cover 19 not protected by the anodes 17, 18 is lined with refractory block 21.

A chlorine gas outlet 22 is fitted through the cover 19 and block 21 and communicates with the space above the electrolyte 16. Direct current is supplied to the connectors 6 and 20. A cover 23 is fitted to the first and second stage reactor compartments, the pump compartment and the product metal storage sump. Refractory block linings 24 are used to protect the undersurface of the cover 23. The covers 19 and 23 are sealed and gas tight. Refractory block lining 25 protects the walls of the reactor compartments 13, 14.

A pair of vertical shafts 26 driven by motors (not shown) project through glands 27 in the cover 23 and are fitted with refractory-clad impellers 28 which have inclined blades adapted to spray upwardly the liquid metal 7 which enters the first and second stage reactor compartments 13, 14 from the electrolysis compartment 11 through passageway 29 which is at such a level that the interface between the cathode metal layer 7 and the electrolyte 16 passes through it. A similar passageway 30 for cathode metal and electrolyte extends between the electrolysis compartment 11 and the pump compartment 12.

A wall or baffle 31 is provided in the electrolysis compartment 11 and extends from the end of the said compartment which is nearest to pump compartment 12, to a point spaced a short distance from the opposite end of the compartment 11. The wall or baffle 31 forms a trough 32 between itself and the adjacent wall of the compartment 11. The passageway 30 communicates with one end of the trough 32. A wall or weir 33 between pump compartment 12 and product metal storage sump 15 controls the metal level throughout the system. A downwardly sloping passageway 34 is provided in the bottom of sump 15 for periodic tapping of product aluminum, the outlet from passageway 34 being normally closed by a removable plug 35.

A passageway 36, through which the cathode metal/electrolyte interface passes, permits flow of electrolyte from the first stage reactor compartment 13 to the second stage reactor compartment 14 and permits flow of cathode metal in the opposite direction. The flow of metal is controlled by a lip 37 which is located inside the second stage reactor compartment 14 and rises above the cathode metal/electrolyte interface. Metal is delivered from the second stage to the first stage by being

splashed against the dividing wall by impeller 28 and then running down inside lip 37 and through passageway 36.

A metal outlet passage 38 is provided to permit flow of metal from the first stage reactor compartment 13 to the pump compartment 12, this passage being located below the surface of the metal. The pump compartment 12 is provided with an electrolyte metering pump 39 of the gas displacement type adapted to deliver electrolyte 16 entering pump compartment 12 through passage 30 at a controlled rate, when so required, through a passageway 40 to the first stage reactor compartment 13. Alchlor vapour is supplied through the main supply pipe 41 and refractory sparger pipes 42 which project downwardly through the cover 23 into the first stage reactor compartment 13 terminating above the surface of the electrolyte.

As illustrative of the process, the cell is filled with sufficient molten aluminum or aluminum alloy 7 to cover the bottom of the electrolysis compartment 11 and give good electrical contact with the lining 4. A metallic reductant, e.g. magnesium, is added and then sufficient molten electrolyte 16 is poured into the cell to cover the bottom of the anodes 17, 18. The molten electrolyte comprises an alkali metal halide and may also include a selection of alkaline earth metal halides and rare earth metal halides. Preferably it contains sodium chloride.

The source of direct current is connected to the cell and electrolysis of the electrolyte 16 in the electrolysis compartment 11 takes place with deposition of metal reductant, e.g. magnesium, in the cathodic layer 7, the metallic reductant entering into solution in the molten aluminum. After a suitable period the electrolyte metering pump 39 and the impellers 28 are started to circulate electrolyte clockwise through the cell as seen in FIGURE 3 and to circulate molten metal anti-clockwise as seen in the same figure.

When the molten metal is circulating through the first and second stage reactor compartments 13, 14 alchlor vapour is fed from the main 41 through the pipe 42 into the atmosphere above the electrolyte in the first stage reactor compartment 13. Pressure of alchlor in the main 41 is maintained at a constant small positive value. This forces the vapour into the reactor chamber 13 until such time as the pressure built up in the gas space of the chamber is sufficient to halt the vapour flow. When this pressure is relieved by further reaction of the alchlor vapour in the gas space with the electrolyte more alchlor will feed from the main 41. The alchlor forms a double salt with the electrolyte, e.g. if the electrolyte is sodium chloride, sodium aluminum chloride is formed.

The electrolyte flowing from the first stage reactor compartment 13 to the second stage reactor compartment 14 through passageway 36 consists of the double salt, e.g. sodium aluminum chloride, and a proportion of the chloride of the metallic reductant, e.g. magnesium chloride.

Molten metal comprising aluminum or aluminum alloy and the metallic reductant, e.g. magnesium, enters the second stage reactor compartment 14 from the electrolysis compartment 11 through passageway 29. In this compartment the reductant concentration in the aluminum is lowered by a reaction between the reductant and the double salt. For example, sodium aluminum chloride reacts with magnesium to yield sodium chloride and magnesium chloride which are recycled through passageway 29 to the electrolysis compartment 11 where the magnesium chloride is electrolysed, the chlorine being discharged through outlet 22 and the magnesium going into solution in the aluminum in the cathode layer. The sodium chloride is recycled to the first stage reactor compartment 13 by the metering pump 39 where it absorbs alchlor as described above to form the double salt sodium aluminum chloride.

The double salt reacts with the residual metallic reductant in the molten metal phase to yield the chloride of the metallic reductant described above as comprising a proportion of the electrolyte circulated from the first

stage reactor compartment 13 to the second stage reactor compartment 14.

Removal of the residual reductant enables substantially pure aluminum to be circulated through passageway 38, pump compartment 12 and passageway 30 to the electrolysis compartment 11. Excess aluminum flows over weir 33 into product metal storage sump 15 to be tapped off from time to time by removal of plug 35.

What we claim is:

1. A process for the production of aluminum and aluminum alloys which comprises electrolysing in an electrolysis zone a fused salt electrolyte containing at least one alkali metal halide, the cathode being molten aluminum or aluminum alloy containing a metal reductant deposited from the electrolyte by electrolysis, transferring the molten aluminum or aluminum alloy and reductant to a reactor zone, reacting a double salt of alchlor with the metallic reductant in the reactor zone, transferring the chloride product of the metallic reductant to the electrolysis zone, re-cycling molten aluminum containing a lower concentration of the metallic reductant back to the electrolysis zone, and discharging the molten metal product from the reactor zone.
2. A process as claimed in claim 1 wherein alchlor as vapour is contacted in the reactor zone with a salt phase capable of absorbing alchlor as a double salt.
3. A process for the production of aluminum and aluminum alloys which comprises electrolysing in an electrolysis zone a fused salt electrolyte containing at least one alkali metal halide and at least one halide selected from the group consisting of the alkaline earth metal halides and the rare earth metal halides, the cathode being molten aluminum or aluminum alloy containing a metal reductant deposited from the electrolyte by electrolysis; transferring the molten aluminum or aluminum alloy and reductant and electrolyte as a molten salt phase to a reactor zone, reacting alchlor with the molten salt to yield a double salt and reacting the double salt with the metallic reductant in the reactor zone to yield the chloride product of the metallic reductant; transferring the chloride product of the metallic reductant to the electrolysis zone, re-cycling molten aluminum containing a lower concentration of the metallic reductant back to the electrolysis zone, and discharging the molten metal product from the reactor zone.
4. A process according to claim 3 wherein alchlor is fed to the first stage of a two-stage reactor zone, the aluminum or aluminum alloy from the first stage being re-cycled to the electrolysis zone and the salt phase containing both the chloride product of the reductant and the double salt being fed to the second stage of said reactor zone to react with fresh molten aluminum or aluminum alloy and reductant from the electrolysis zone.
5. A process as claimed in claim 4 wherein the salt phase containing the chloride product of the reductant and substantially denuded of alchlor in the second stage is re-cycled to the electrolysis zone.
6. A process for the production of aluminum and aluminum alloys which comprises electrolyzing a fused salt electrolyte containing at least one alkali metal halide, using as cathode a molten metal or alloy which contains in solution a metallic reductant deposited from the electrolyte, and contacting the molten metal or alloy and the contained metallic reductant with a double salt of alchlor, the reaction between the metallic reductant and the double salt of alchlor being effected in two stages, in which process the electrolyte and the molten metal are transferred from the electrolysis zone to the reactor zone in counter-current flow, the alchlor being fed to the first stage of the reactor zone, the electrolyte being fed initially to the first stage of the reactor zone and thence to the second stage of the reactor zone and the molten metal being fed initially to the second stage of the reactor zone and thence to the first stage of the reactor zone.

7. A process for the production of aluminum and aluminum alloys wherein a fused salt electrolyte containing at least one alkali metal halide is electrolyzed using a cathode of a molten metal or alloy, in which the electrolyte comprises a halide of a metallic reductant for aluminum chloride which reductant is soluble in the cathode, the metallic reductant being deposited by electrolysis from the electrolyte and dissolved in the cathode, and the cathode metal or alloy and the contained reductant being brought into contact with a double salt of alchlor.

8. A process according to claim 7, in which the molten salt electrolyte is electrolyzed in an electrolysis cell and the cathode metal or alloy and the contained metallic reductant are transferred to a reactor in which a double salt of alchlor is contacted with the metallic reductant to produce a chloride of the reductant, which chloride is transferred to the electrolysis cell, the molten metal or alloy containing aluminum and a correspondingly lower concentration of metallic reductant, part of which is fed back to the electrolysis cell and part of which is discharged from the reactor as the molten metal product.

9. A process according to claim 7, in which the cathode comprises molten aluminum or aluminum alloy.

10. A process according to claim 7, in which the electrolyte contains at least one halide of a metal selected from the group consisting of the alkaline earth metals and the rare earth metals.

11. A process according to claim 7, in which alchlor is contacted with a salt phase which is able to absorb the alchlor to thereby form therewith a double salt.

12. A process as claimed in claim 11, in which the alchlor is at a superatmospheric pressure in the reactor.

13. A process as claimed in claim 7, in which the metallic reductant is magnesium.

14. A process as claimed in claim 7, in which the metallic reductant is lithium.

15. A process according to claim 7, in which reaction between the metallic reductant and double salt of alchlor is carried out in a reactor having two sections.

16. A process according to claim 15, in which alchlor is fed to the first section of the reactor and contacted with salt phase to form a double salt of alchlor; and a portion of the salt phase and the contained double salt is transferred to the second section.

17. A process according to claim 15, in which cathode metal or alloy and the contained metallic reductant is transferred from the electrolysis cell to the second section and then to the first section of the reactor so as to contact the salt phase thereby to produce aluminum or aluminum alloy, a portion of which is transferred from the first section of the reactor to the electrolysis cell.

18. A process according to claim 17, in which the salt phase from the second stage of the reactor, is transferred to the electrolysis cell.

19. A process according to claim 7, in which the molten metal or alloy from the electrolysis cell and the double salt of alchlor are brought together in counter-current flow.

20. A process as claimed in claim 8, in which the molten metal or alloy in the reactor is agitated.

#### References Cited

##### UNITED STATES PATENTS

|           |         |         |       |           |
|-----------|---------|---------|-------|-----------|
| 362,441   | 5/1887  | Gratzel | ----- | 204—67    |
| 387,876   | 8/1888  | Heroult | ----- | 204—67 XR |
| 2,742,418 | 4/1956  | Padgett | ----- | 204—71 XR |
| 2,919,234 | 12/1959 | Slatin  | ----- | 204—71 XR |

##### FOREIGN PATENTS

|         |         |                |
|---------|---------|----------------|
| 16,794  | 10/1889 | Great Britain. |
| 757,908 | 9/1956  | Great Britain. |

JOHN H. MACK, Primary Examiner

D. R. VALENTINE, Assistant Examiner

U.S. CL. X.R.

204—67, 68